

R. A. LEWIS, W. R. SHIMER & W. J. THOMAS,  
TREATMENT OF STEEL RAILS,  
APPLICATION FILED MAY 15, 1915.

1,285,748.

Patented Nov. 26, 1918.



Fig. 1

Fig. 2



By their Attorney *Roy A. Lewis*  
*W. Robert Shimer*  
and  
Claimant, *William J. Thomas*

# UNITED STATES PATENT OFFICE.

ROY A. LEWIS, WILLIAM ROBERT SHIMER, AND WILLIAM J. THOMAS, OF BETHLEHEM, PENNSYLVANIA, ASSIGNORS TO BETHLEHEM STEEL COMPANY, OF SOUTH BETHLEHEM, PENNSYLVANIA, A CORPORATION OF PENNSYLVANIA.

## TREATMENT OF STEEL RAILS.

1,285,748.

Specification of Letters Patent. Patented Nov. 26, 1918.

Application filed May 15, 1915. Serial No. 28,281.

To all whom it may concern:

Be it known that we, ROY A. LEWIS, WILLIAM ROBERT SHIMER, and WILLIAM J. THOMAS, all citizens of the United States, 5 and residents of Bethlehem, Northampton county, Pennsylvania, have jointly invented new and useful Improvements in the Treatment of Steel Rails, of which the following is a specification, reference being had to the 10 accompanying drawings, in which—

Figure 1 represents a diagrammatic arrangement illustrating an apparatus suitable for carrying out our invention, and Fig. 2 is a section on lines II—II of Fig. 1. 15 Our invention relates to the treatment of rails, and consists particularly in the heat treating of rails after the last forming operation and while they retain part of the heat of the final rolling or forming operation. 20 Our invention also consists in the modes of treatment which we shall hereinafter describe and claim.

A typical manner of carrying out our invention in connection with the apparatus 25 shown in the drawings is as follows:

The rail is preferably rolled from a re-heated bloom, in order that it may leave the rolls at a high finishing temperature, so that it may be free from internal strains after 30 the rolling operation has been completed. We have found that the rail is at a temperature of between 1700° and 2075° F. as it leaves the finishing rolls, and is cooled to between 1600° and 1950° F. by the time it 35 leaves the hot saw. The rail is then passed through an air spray A, remaining therein for from five to ten minutes, in order to cool the rail rapidly and thereby prevent, as far as possible, the formation of free ferrite or 40 laminated pearlite, and retains, as far as is possible, the structure of the metal in the condition in which it comes from the finishing rolls. As the rail is cooled rapidly to well below the critical or calecence point 45 (which is about 1370° F.), that is, to about 1000° to 1100° F., the separation of the constituents, free ferrite, laminated pearlite and grain growths, is prevented to a large degree and the homogeneous character of the metal 50 is substantially maintained.

The rail, after cooling, is conveyed to a continuous re-heating furnace B, in which it remains for a period of preferably between forty-five minutes to an hour. The charg-

ing end of the furnace is about 1300° F., and 55 as the rail is advanced the furnace temperature increases, so as to bring the rail, during the latter part of its travel, to approximately between 1400° and 1500° F. This 60 temperature is maintained so as to insure a thorough and uniform heating of the rail, so that, when the rail leaves the furnace, all 65 of its parts will have reached approximately the same temperature, at which the iron and carbon will exist in the rail in a homogeneous solid solution.

As the rail is discharged from the furnace it is again cooled quickly, preferably in oil or any other suitable cooling medium, at C. By cooling quickly the steel is hardened 70 and the solid solution of iron and carbon is maintained as far as possible without change. The cooling is preferably effected in three or four minutes, and the temperature is reduced from above the critical point to preferably 75 between 600° and 1000° F., depending largely on the cooling medium used. If oil is used, it is cooled to or below 600° F.

After the second cooling, and while the rail still contains an appreciable amount of 80 heat, it is carried to an annealing furnace D, in which the temperature of the charging end is about 1000° F. and is increased gradually toward the middle of the furnace, and from this point to the discharge end 85 the furnace will be at a temperature necessary to heat the rail uniformly to between 1000° to 1250° F., (that is, below the recalcence point, which is about 1250° F.) depending on the composition of the rails and the required physical and wearing qualities. 90

It is important that the heat treating of the rails take place immediately after the rails have been rolled, so that the high finishing temperature may be utilized. By 95 using an air blast or other cooling medium by which the rail is cooled quickly, much time is saved in completing the treatment of the rail, and it must be cooled quickly in order to prevent, as far as possible, the separation of free ferrite and grain growth, which would occur if the rail were allowed to cool in the usual manner.

As the rail is preferably not cooled to 100 below 1000° F., it being only necessary to cool it below the critical point, it can be re-heated quickly in the re-heating furnace, which is for the purpose of raising the steel 105

to a uniform temperature above the critical point and thereby render its structural composition uniform. It is necessary to cool quickly the second time in order to harden, 5 refine and maintain the solid solution of iron and carbon, and it is again cooled to below the critical temperature, but not entirely cooled, since it is desired to utilize the heat of the rail in the subsequent annealing operation. The second cooling acts 10 both to harden and refine the rail, the final hardness depending on the rate of cooling and the temperature at which the rail is heated in the annealing furnace.

15 In the annealing furnace the rail remains in the furnace a sufficient length of time so as to be uniformly heated throughout and is relieved of strains, and is heated to the desired temperature to give it the requisite 20 strength, hardness and ductility.

We have found that rails containing, (1) .61% carbon, .68% manganese; (2) .71% carbon, .76% manganese, and with silicon, sulfur and phosphorus in the percentages 25 usually found in rail steel, treated in accordance with our invention, have given the following results in comparison with untreated rails of the same composition:

(1) .61% carbon, .68% manganese.

|                                  | Treated.     | Untreated.   |
|----------------------------------|--------------|--------------|
| Tensile strength per sq. in..... | 130,000 lbs. | 107,500 lbs. |
| Elastic limit per sq. in.....    | 80,000 "     | 54,000 "     |
| Elongation.....                  | 17.5%        | 15%          |
| Reduction in area.....           | 43.3%        | 24.08%       |
| Brinell hardness No.....         | 265          | 214          |

(2) .71% carbon, .76% manganese.

|                                  | Treated.     | Untreated.   |
|----------------------------------|--------------|--------------|
| Tensile strength per sq. in..... | 138,000 lbs. | 120,000 lbs. |
| Elastic limit per sq. in.....    | 88,000 "     | 66,000 "     |
| Elongation.....                  | 19.5%        | 13.5%        |
| Reduction in area.....           | 48.8%        | 22.3%        |
| Brinell hardness No.....         | 260          | 227          |

45 the treated steel showing the following increases over the untreated steel:

|                                  | Specimen No. 1. | Specimen No. 2. |
|----------------------------------|-----------------|-----------------|
| Tensile strength per sq. in..... | 22,500 lbs.     | 18,000 lbs.     |
| Elastic limit per sq. in.....    | 25,000 "        | 22,000 "        |
| Elongation.....                  | 2.5 %           | 6 %             |
| Reduction in area.....           | 19.22%          | 26.5%           |
| Brinell hardness No.....         | 51              | 23              |

50 In both instances the treated steel shows much greater strength and higher elastic limit and is much more ductile, although considerably harder, than the untreated steel.

55 It will be seen that by our process the rails can be run through the furnace in large quantities and in a comparatively short period of time. The first cooling step and the first re-heating step are desirable,

since by employing them we are enabled to heat the rail at a uniform temperature above the critical point, so that, when the rails are cooled in the bath C, all of the parts of the rail will be affected uniformly. We have 70 found, however, that good results may be obtained by eliminating the re-heating treatment in the furnace B and one of the cooling treatments; that is, we take the rail as it comes from the hot saw and cool it 75 quickly to about 1000° F. and pass it directly into the annealing furnace D, but the rails treated by this method are not as uniform as those treated by the method which we have described above, for the reason that, as the rail comes from the rolling operation, its flanges and webs will have cooled to a greater extent than have the head and base of the rail, and hence, in the resulting product, the steel is not nearly so 85 uniform as when the re-heating operation is included in carrying out our process.

80 The terms and expressions which we have employed are used as terms of description and not of limitation, and we have no intention, in the use of such terms and expressions, of excluding any equivalent for the features which we have described, but recognize that various modifications are possible within the scope of the invention 95 claimed.

90 We claim is:

1. The method of heat-treating rails, which consists in taking a highly heated rail as it comes from the final forming operation, cooling it quickly to below 1300° F. and above 1000° F., conveying it to a heating furnace and heating it therein until it reaches a uniform temperature above 1400° F. and below 1500° F., then cooling 100 rapidly to between 1000° and 600° F., and then passing it through an annealing furnace, in which the rail is uniformly heated to between 1000° F. and 1200° F., and then cooling.

105 2. The method of heat-treating rails, which consists in taking a highly heated rail as it comes from the final forming operation and while its temperature is above 1600° F. and below 2075° F., cooling it 110 quickly in an air spray to below 1300° F. and above 1000° F. to prevent the separation of free ferrite, then passing the rail through a heating furnace and heating the rail in all of its parts to a temperature not less than 1400° F., maintaining the rail at such temperature for a determinate period of time, and cooling quickly to below 1000° F., re-heating to not less than 1000° F. but below 1200° F. and maintaining it at such 115 temperature for a determinate period of time, and then cooling.

120 3. The method of heat-treating rails, which consists in taking a highly heated rail as it comes from the final forming op- 125

eration, and while the temperature is above 1600° F. and below 2075° F., cooling it quickly to below 1000° F., then passing the rail through a heating furnace and heating it therein until it reaches a uniform temperature above 1370° F. and below 1500° F. while keeping all of its parts in the passage therethrough accessible to the heat, maintaining the rail at a uniform heat for 10 a determinate period of time, and then cooling.

4. The method of heat-treating rails, which consists in taking a highly heated rail as it comes from the last forming operation, cooling it quickly to below 1000° F. to prevent the formation of laminated pearlite, conveying the rail to a heating furnace and heating it therein uniformly to between 1400° to 1500° F. to prevent the separation of free ferrite and for hardening, and then passing the rail through an annealing furnace in which the rail is heated uniformly to between 1000° F. and 1200° F. to soften, toughen and relieve it of 25 strains, and then cooling.

5. The method of heat-treating rails, which consists in taking a highly heated rail

as it comes from the final forming operation, cooling it quickly in an air blast to below 1000° F., conveying it to a heating furnace and heating it therein until it reaches a uniform temperature above 1400° F., then cooling rapidly in an oil bath and then passing it through an annealing furnace, in which the rail is uniformly heated to between 1000° F. and 1200° F., and finally cooling.

6. The method of producing a hard and tough steel rail, which consists in taking a highly heated rail as it comes from the final forming operation, and cooling the surface of the rail quickly by means of an elastic fluid to a temperature below 1000° F. to prevent the formation of grain growths, then passing the rail through a heating furnace and heating the rail therein in all of its parts to a temperature above 1400° F. to get the rail in proper condition for hardening, cooling, and then annealing at a temperature below 1200° F. and above 1000° F.

ROY A. LEWIS.  
W. ROBERT SHIMER.  
WILLIAM J. THOMAS.